

# UNITED STATES PATENT OFFICE.

CARL D. HOCKER, OF EAST ORANGE, NEW JERSEY, ASSIGNOR TO WESTERN ELECTRIC COMPANY, INCORPORATED, OF NEW YORK, N. Y., A CORPORATION OF NEW YORK.

## LIQUID COATING COMPOSITION. REISSUED

1,422,861.

Specification of Letters Patent.

Patented July 18, 1922.

No Drawing.

Application filed December 11, 1919. Serial No. 344,177.

To all whom it may concern:

Be it known that I, CARL D. HOCKER, a citizen of the United States, residing at East Orange, in the county of Essex, State 5 of New Jersey, have invented certain new and useful Improvements in Liquid Coating Compositions, of which the following is a full, clear, concise, and exact description.

This invention relates to the production of 10 suitable resinous compositions which may be employed as the base in the manufacture of varnishes, impregnating compounds, lacquers, enamels, japans, and the like. More particularly it has to do with the use of such 15 coating when heat is applied thereto to facilitate the drying thereof.

In enameling or japanning electrical conductors or other metallic surfaces for example, either for electrical insulation or atmospheric protection, many compounds 20 composed of resinous or oily materials, or both combined with volatile solvents or vehicles have been used. The usual method 25 of application has been to apply the composition while in the condition of a thin liquid, thereafter removing the solvent or vehicle by increasing the temperature. The tendency in such a process is to produce a 30 more or less non-continuous coating due to the impossibility of removing the solvent uniformly. The solution of such a problem would seem to lie in using a composition which after application with the aid of heat 35 will undergo a chemical change, thereby converting part of the solvent or vehicle used into a solid which will form part of the finished coating.

An object of the invention is to produce 40 a liquid coating composition, which after application with the aid of heat, converts the prepared liquid coating composition into a semi-solid through chemical action; and with continued heating, such as usually applied to bake enamels and japans, forms a 45 hard, firm, continuous and durable coating.

It has been found that such compositions 50 may be formed by combining under the proper conditions a resin, such as Congo copal, shellac, Manila copal, etc., one or 55 more free fatty acids and a polyacid alcohol such as glycerine. In carrying out the preparation of such a compound, the resin and

free fatty acids are mixed in suitable proportions until, with the aid of heat, a uniform homogeneous mass is obtained. This condition having been arrived at, the polyacid alcohol is added and the temperature increased until the mass again becomes homogeneous. For example, if 150 parts of congo copal are added to 500 parts of a mixture of 60 free fatty acids such as is derived from a vegetable oil by the saponification thereof, 112½ parts of glycerine will be required to give the final product the desired consistency. When the mass has become cool, a thick 65 syrupy liquid is obtained which contains about 20 per cent of its weight as resin.

The compound so produced possesses the property of gelatinizing upon the further application of heat without the addition of 70 other substances. This feature in itself will widen the field of application of compositions prepared from the materials heretofore mentioned.

While the above method is sufficient to 75 produce the desired result, it is somewhat expensive because of the large amount of free fatty acid and polyacid alcohol required. By substituting a vegetable oil, say castor oil, for example, for part of the glycerine and part of the acid, the cost of the material will be considerably decreased and the product will be identical for practical purposes with that produced in the afore-mentioned manner. In carrying out this process, 80 which is the preferred method of producing the liquid coating composition, 150 parts of congo copal are mixed with 100 parts of the free fatty acids, ricinoleic, dihydroxystearic 85 and stearic, which are derivable from castor oil by saponification. The temperature having been raised until a homogeneous mass is obtained, 37½ parts of glycerine and 510 parts of castor oil are then added. The heating is then continued until a certain predetermined condition is attained. The composition 90 will then be in such a state that further heating will cause gelatinization.

Before such gelatinization is carried out however, the composition is applied to the 100 surface which is to be coated. It is desirable, in some cases at least, to add organic solvents, such as kerosene and the like, in order to render the composition more liquid.

When a smooth, uniform covering has been secured, heat is applied thereto in such a manner that a gradual thickening of the fluid coating takes place. The temperature 5 is then increased until solidification occurs.

It is to be understood that although Congo copal and shellac have been mentioned herein specifically, it is intended to include any resin which has the property of forming 10 a gelatinous product with a polyacid alcohol. In referring to vegetable oils or fatty oils, all oils which will, upon saponification yield one or more fatty acids are included. Some of the oils which have been used are: 15 Chinese wood oil, corn oil, castor oil, linseed oil, soya bean oil, rapeseed oil, sesame oil, cotton-seed oil and peanut oil.

In order that it may be understood what acids are intended to be included as belonging 20 to the fatty acid class, a word of explanation is considered necessary. Various textbooks which contain matter relating to the chemical composition of such substances, differ in their classification of the fatty 25 acids. As used in this specification, the term "fatty acids" is considered to include any and all classes embraced by the following outline.

1. Acids of the acetic series,  $C_nH_{2n}O_2$ .
2. Acids of the oleic series,  $C_nH_{2n-2}O_2$ .
3. Acids of the series,  $C_nH_{2n-4}O_2$ , which includes the open chain and cyclic acids.
4. Acids of the linoleic series,  $C_nH_{2n-6}O_2$ .

5. Acids of the clupanodonic and the  $C_nH_{2n-8}O_2$  series.

6. Hydroxylated and carboxylated acids of any of the above classes.

What is claimed is:

1. A liquid coating composition resulting from a combination comprising glycerine, resin, and free fatty acid.

2. A liquid coating composition resulting from a combination comprising glycerine, resin, free fatty acid and vegetable oil.

3. A liquid coating composition resulting from a combination comprising glycerine, congo copal, free fatty acid and castor oil.

4. The process of making a liquid coating composition which comprises treating resin with free fatty acid, and combining glycerine with the product so formed.

5. The process of making a liquid coating composition which comprises treating resin with free fatty acid, and combining glycerine and vegetable oil with the product so formed.

6. The process of making a liquid coating composition which comprises treating congo copal with free fatty acid and combining glycerine and castor oil with the product so formed.

In witness whereof, I hereunto subscribe my name this 10th day of December, A. D., 1919.

CARL D. HOCKER.